

# United States Patent [19]

Shiba et al.

[11] 3,895,948

[45] July 22, 1975

[54] **SILVER HALIDE LIGHT-SENSITIVE MATERIAL CONTAINING A HETEROCYCLIC THIONE AND A POLYALKYLENE OXIDE**

[75] Inventors: **Keisuke Shiba; Seiiti Kubodera; Reiichi Ohi; Tadao Shishido; Nobuo Yamamoto; Takeo Sakai**, all of Kanagawa, Japan

[73] Assignee: **Fuji Photo Film Co., Ltd.**, Minami Ashigara, Japan

[22] Filed: **Dec. 29, 1972**

[21] Appl. No.: **319,815**

[30] **Foreign Application Priority Data**

Dec. 28, 1971 Japan ..... 47-3037

[52] U.S. Cl. ..... 96/76 R; 96/95; 96/107; 96/66.3

[51] Int. Cl. ..... G03c 1/06; G03c 1/28

[58] Field of Search ..... 96/107, 109, 95, 66.3, 96/66.5, 76 R

[56] **References Cited**

UNITED STATES PATENTS

|           |         |              |        |
|-----------|---------|--------------|--------|
| 2,772,164 | 11/1956 | Allen et al. | 96/109 |
| 2,956,876 | 10/1960 | Spath        | 96/109 |
| 3,081,170 | 3/1963  | Rauch et al. | 96/109 |
| 3,161,520 | 12/1964 | Rauch et al. | 96/109 |

|           |         |                  |        |
|-----------|---------|------------------|--------|
| 3,294,540 | 12/1966 | Goffe            | 96/107 |
| 3,345,175 | 10/1967 | Hayakawa et al.  | 96/109 |
| 3,397,987 | 8/1968  | Luckey et al.    | 96/109 |
| 3,433,640 | 3/1969  | Nishio et al.    | 96/107 |
| 3,518,085 | 6/1970  | Milton et al.    | 96/109 |
| 3,692,527 | 9/1972  | Von König et al. | 96/109 |
| 3,708,303 | 1/1973  | Salesin          | 96/107 |

Primary Examiner—Won H. Louie, Jr.  
Attorney, Agent, or Firm—Sughrue, Rothwell, Mion, Zinn and Macpeak

[57] **ABSTRACT**

A silver halide light-sensitive material which contains at least one compound selected from the group of compounds represented by the following general formula (I):



and at least one polyalkylene oxide derivative in a silver halide emulsion layer or a layer adjacent thereto. In the above formula, Q represents the atoms necessary to form heterocyclic ring and R represents an alkyl group, an aryl group or a hetero group.

**10 Claims, 5 Drawing Figures**



**FIG. 1****FIG. 3****FIG. 5****FIG. 2****FIG. 4**

**SILVER HALIDE LIGHT-SENSITIVE MATERIAL  
CONTAINING A HETERO CYCLIC THIONE AND A  
POLYALKYLENE OXIDE**

**BACKGROUND OF THE INVENTION**

1. Field of the Invention

The present invention relates to a silver halide light-sensitive material and, more particularly, it relates to a lithographic light-sensitive material which provides an image of a high edge gradient.

2. Description of the Prior Art

In a photographic image when a blackened area and non-blackened area are contiguous to each other the ratio of change in optical density versus the distance in a direction at right angles to the tangent is referred to as the edge gradient. In general, the higher the edge gradient the sharper the image. In particular, a light-sensitive material capable of providing an image having a high edge gradient is useful, e.g., as a lithographic light-sensitive material for use in photographic plate-making processes wherein a dot image is prepared using a glass screen or a contact screen. For the purpose of developing these light-sensitive materials so as to obtain an image with high edge gradient a special developer having a high pH and containing hydroquinone as a developing agent and a small amount of sulfite (called an "infectious developer") is used.

On the other hand, it is known that when a polyalkylene oxide derivative, such as the addition polymer of 1 molecule of sorbitan monolaurate with about 20 molecules of ethylene oxide, is used in a light-sensitive material a rise in contrast is caused.

However, an emulsion wherein a polyalkylene oxide derivative is used has the defect that prolonged development is required in order to obtain high contrast.

In addition, an emulsion containing a polyalkylene oxide derivative requires a long initial development before the start of infectious development, though such an initial development provides, once infectious development starts, high contrast by markedly strengthening the infectious development. Therefore, extremely low contrast gradation obtained in the initial development co-exists with high contrast gradation, which results in insufficient "toe-gradation" (see FIG. 1, curve 11). This results from the fact that the polyalkylene oxide derivative makes the starting point of the infectious development irregular with respect to the individual silver halide grains contained in the emulsion.

To the light-sensitive material in accordance with the present invention can be applied the art of spectral sensitization. Most of sensitizing dyes used for spectral sensitization make the toe-gradation worse, which has also been the case with the aforesaid polyalkylene oxide derivatives. In such cases, even when high contrast is obtained in the half tone image, good dots with sharp edges cannot be obtained by comparatively short time development usually practiced (shorter than 3 minutes) in the case of recording dot images. Good results are obtained with such short time development in the present invention, however.

**SUMMARY OF THE INVENTION**

A primary object of the present invention is, therefore, to provide an emulsion capable of providing high edge gradient with a comparatively short development time.

Another object of the present invention is to provide an emulsion capable of providing dots having good toe-gradation, i.e., in the plot of Density vs. Exposure (log E), the characteristic curve continues into the region of decreasing exposure with constantly decreasing gradient until at a point the gradient becomes zero, that is, the curve becomes parallel to coincident with the log E axis. The region, where the curve starts to flatten, is referred to in the art as the toe of the characteristic curve.

A further object of the present invention is to improve the deterioration of toe-gradation caused by the use of certain sensitizing dyes without a reduction in light sensitivity and while providing a supersensitizing action.

Still a further object of the present invention is to render uniform the size and quality of individual dots in the density region wherein the dot size is small.

It has been found that the above objects of the present invention can be attained by using a silver halide photographic emulsion containing at least one polyalkylene oxide derivative and at least one compound represented by general formula (I):

25

30

35



wherein Q represents the atoms necessary to form a heterocyclic ring (which heterocyclic ring may be substituted) and R represents an alkyl group, an aryl group or a heterocyclic group.

**BRIEF DESCRIPTION OF THE DRAWINGS**

FIG. 1 is a characteristic curve with optical density (D) on the vertical axis and exposure amount (log E) horizontally.

FIGS. 2-5 are curves showing the relationship between the distance [ L (unit:micron) ]-optical density in the edge portion of a dot.

45 **DETAILED DESCRIPTION OF THE INVENTION**

In the above general formula (I), Q represents the atoms necessary to complete a heterocyclic ring (which ring may be substituted), such as benzothiazolin-2-thione ring, 6-methyl-benzothiazolin-2-thione ring, 6-ethyl-benzothiazolin-2-thione ring, 6-methoxy-benzothiazolin-2-thione ring, 6-chloro-benzothiazolin-2-thione ring, 4,5-tetramethylenethiazolin-2-thione ring, 4,5-trimethylenethiazolin-2-thione ring, naphthothiazolin-2-thione ring, thiazolidin-2-thione ring (e.g., thiazolidin-2-thione ring, 4-methylthiazolidin-2-thione ring, etc.), imidazolin-2-thione ring (e.g., 1,3-dimethylimidazolin-2-thione ring, 1,3-diethylimidazolin-2-thione ring, etc.), selenazolidin-2-thione ring (e.g., selenazolidin-2-thione ring, 4-methylselenazolidin-2-thione ring, etc.), a 1,3,4-thiadiazolin-2-thione ring (e.g., 1,3,4-thiadiazolin-2-thione ring, 5-methyl-1,3,4-thiadiazolin-2-thione ring, 5-ethylthio-1,3,4-thiadiazolin-2-thione ring, 5-{2-(4-phenyl-5-thio-1,3,4-thiadiazolin-2-yl)-mercaptoethylthio}1,3,4-thiadiazolin-2-thione ring, etc.), 1,3,4-selenadiazolin-2-thione ring (e.g., 1,3,4-selenadiazolin-2-thione ring, 5-ethyl-1,3,4-selenadiazolin-2-thione ring, etc.), 4-

5 selenazolin-2-thione ring (e.g., 4-selenazolin-2-thione ring, 4-methyl-4-selenazolin-2-thione ring, 4-phenyl-4-selenazolin-2-thione ring, etc.), 1,2-dihydropyridin-2-thione ring (e.g., 1,2-dihydropyridin-2-thione ring, 6-ethyl-1,2-dihydropyridin-2-thione ring, etc.), benzoxazolin-2-thione ring (e.g., benzoxazolin-2-thione ring, 6-ethylbenzoxazolin-2-thione ring, 6-methoxybenzoxazolin-2-thione ring, 5-methylbenzoxazolin-2-thione ring, etc.), benzimidazolin-2-thione ring (e.g., 1,3-dimethylbenzimidazolin-2-thione ring, 1,3-di-n-propylbenzimidazolin-2-thione ring, 1,3-di-n-decylbenzimidazolin-2-thione ring, 1,3-di-benzylbenzimidazoline-2-thione ring, 5-chloro-1,3-dimethylbenzimidazolin-2-thione ring, 5-methyl-1,3-di-benzylbenzimidazolin-2-thione ring, etc.), benzoselenazolin-2-thione ring (e.g., benzoselenazolin-2-thione ring, 6-ethylbenzoselenazolin-2-thione ring, 6-methoxybenzoselenazolin-2-thione ring, 6-chlorobenzoselenazolin-2-thione ring, etc.), 1,2-dihydroquinolin-2-thione ring (e.g., 1,2-dihydroquinolin-2-thione ring, 6-methyl-1,2-dihydroquinolin-2-thione ring, 6-chloro-1,2-dihydroquinolin-2-thione ring, etc.), and the like.

25 The group R includes unsubstituted or hydroxy-aryl-, morpholino- or like group-substituted alkyl group having 1-13 carbon atoms, preferably, 1-6 carbon atoms, such as a methyl group, ethyl group, propyl group, hexyl group, decyl group, hydroxyethyl group, benzyl group and a morpholinoethyl group, etc; unsubstituted or alkyl-, alkoxy-, halogen-, or the like group-30 substituted aryl groups, such as a phenyl group, 2-methylphenyl group, 4-methoxyphenyl group, and a 4-chlorophenyl group, etc.; heterocyclic ring group, such as 2-pyridyl group, a dipyridyl group and the like.

35 Specific examples of several preferred compounds used in the present invention include the following compounds:

m.p. 55°C



m.p. 149°C



m.p. 190°C



m.p. 87°C



m.p. 130°C



m.p. 81-82°C



5

(I-10)



m.p. 102°C

(I-16)

6



m.p. 166°C

(I-11)



m.p. 96°C

(I-17)



m.p. 113°C

(I-12)



m.p. 114°C

20

25

(I-13)



m.p. 162°C

30

35

40

(I-18)



30

(I-14)



m.p. 82°C

(I-19)



50

55

(I-15)



m.p. 119°C

(I-20)



60

65

65

65

65





9

(I-32)



10

(I-37)



(I-33)



m.p. 625°C

15 (I-38)



(I-34)



(I-39)



(I-35)



(I-36)



Although the above-illustrated compounds can be synthesized according to conventionally known processes, synthesis examples of the above compounds are given below.

### Synthesis Example 1 (Compounds I-1 through I-8)

These compounds can be synthesized according to the process described in the Journal of The Chemical Society, 1939, pages 473 - 476, using 2-mercaptopbenzothiazole as a starting material.

### Synthesis Example 2 (Compounds I-9 through I-17)

The compounds can be synthesized according to the process described in the Journal of The Chemical Society, 1949, pages 1,503 - 1,509, by reacting dithiocarbamate with an alpha-haloketone.

Compounds I-18-I-29 can be prepared by the procedure of Synthesis Example 1, in which the starting material is changed.

65 Compounds I-30~I-39 can be prepared by the procedure of Synthesis Example 2, in which the starting materials are changed.

Compounds I-1~I-39 are well known in the art.

As illustrative of the polyalkylene oxide derivatives used in the invention there are addition polymerization products between alkylene oxides such as ethylene oxide or propylene oxide and a compound such as water, an aliphatic alcohol, an aromatic alcohol, glycols, fatty acids, organic amines and a dehydrated compound of a hexitol derivative; condensates of a polyalkylene oxide with a compound such as just described; or block co-polymers of various alkylene oxides such as ethylene oxide- propylene oxide block copolymers as described in U.S. Pat. No. 3,516,380, etc. Additional examples of such materials are described in, for example, U.S. Pat. Nos. 2,400,532; 3,294,537; and 3,294,540, French Pat. Nos. 1,491,805; 1,596,673, Japanese Patent Publication No. 23466/65, and the like.

The polyalkylene oxide derivatives used in the present invention are those having a molecular weight of from 500 to 12,000, most preferably from 800 to 6,000. Specific examples thereof include the following:

a.



25

b.



c.



wherein  $b$  represents an integer of 14 - 55 and  $a+c$  is an integer of 4 - 210. Such materials are available from Wyandotte Chemical Co. under the trade name "Pluronic L-44, L-61, L-62, L-64, L-68, L-81, P-65, P-75, F-88," etc. In Pluronic L-68, for example, the molecular weight is 8,750,  $b=32$  and  $a+c=159$ ; in Pluronic P-75, the molecular weight is 4,100,  $b=37$  and  $a+c=51$ ; and in Pluronic F-88, the molecular weight is 11,250,  $b=41$  and  $a+c=204$ .

d.  $\text{HOCH}_2\text{CH}_2\text{O}(\text{CH}_2\text{CH}_2\text{O})_{50}\text{CH}_2\text{CH}_2\text{OH}$ 

e.



45

General formula (II)



wherein  $Z_1$  represents the atoms necessary to form a tetrazole nucleus, pyrrolidine nucleus, pyridine nucleus, thiazole nucleus, thiazoline nucleus, selenazole nucleus, selenazoline nucleus, oxazole nucleus, oxazoline nucleus, indolene nucleus or imidazole nucleus,  $L$  represents a methine chain, such as an unsubstituted or a substituted methine group, for example, an alkyl(- $\text{C}_1\text{--C}_6$ )-substituted methine group or a phenyl-substituted methine group,  $Y_1$  represents an oxygen atom, sulfur atom or  $=\text{N}-\text{R}_6$  (wherein  $\text{R}_6$  represents an alkyl group having 1 - 6 carbon atoms, e.g., methyl, ethyl, propyl, cyanoethyl, allyl, carboxyethyl, dimethylaminoethyl, benzyl group, etc., an aryl group such as a phenyl group or p-sulfonylphenyl group)  $n$  represents 0 or 1,  $R_4$  and  $R_5$  represent an alkyl group (e.g., methyl, ethyl, carboxyethyl, carboxybutyl, sulfoethyl, sulfopropyl, allyl, morpholinoethyl, acetoxypropyl, benzyl group, etc.), aryl group such as a phenyl group, a tolyl group, a pyridyl group or like group,

General formula (III)



wherein  $l + m + n =$  about 20, and

f.



The compounds used in the invention and represented by the general formula (I) are characterized by the presence of a thioether functional group. It is important in the invention that compound (I) has a thi-

oketone functional group and the substituent  $R$  be a substituent other than a hydrogen atom. Such a compound gives effective results when combined with a polyalkylene oxide derivative. Since in these compounds  $R$  is not hydrogen the compounds cannot form a tautomeric isomer having a mercapto group, and no reduction in sensitivity is encountered upon the use of such compounds. On the contrary, these compounds supersensitive with most generally used simple merocyanine dyes, dimethine merocyanine dyes and carbocyanine dyes, and hence they raise the sensitivity without increasing the fog formation.

The silver halide photographic emulsions in accordance with the present invention can be spectrally sensitized, for example, by one or more sensitizing dyes represented by general formula (II) or (III):

General formula II

50

wherein  $A$  represents a hydrogen atom, lower alkyl group having not more than 3 carbon atoms, such as methyl, ethyl, propyl group, etc.,  $Z_2$  and  $Z_3$  represent the atoms necessary to form an aromatic ring of the benzene series, such as 5-phenylbenzoxazole, 5-chlorobenzoxazole, 5-methoxycarbonylbenzoxazole, 5-acetoxybenzoxazole, 5-chlorobenzothiazole, 5-chloro-6-methylbenzothiazole, 5-methylbenzothiazole, benzoselenazole, 5-methylbenzoselenazole, 5,6-

dichlorobenzimidazole, 5-chloro-6-methylsulfonylbenzimidazole, or the atoms necessary to form an aromatic ring of the naphthalene series, such as naphthothiazole, naphthoselenazole or naphthoimidazole, the terms benzene and naphthalene series thus including both unsubstituted or substituted benzene and naphthalene, for example, the substituent can be an alkyl group, generally a C<sub>1</sub>-C<sub>13</sub>, preferably a C<sub>1</sub>-C<sub>6</sub> alkyl group, a halogen atom or a phenyl group, Y<sub>2</sub> and Y<sub>3</sub> represent an oxygen atom, sulfur atom, selenium atom, or —NR<sub>7</sub>(R<sub>7</sub> being a (C<sub>1</sub>-C<sub>13</sub>) alkyl group, preferably a C<sub>1</sub>-C<sub>6</sub> alkyl group such as methyl, ethyl, allyl, acetoxyethyl, cyanoethyl group, etc.), R<sub>5</sub> and R<sub>6</sub> represent an alkyl group having not more than 6 carbon atoms, such as methyl, ethyl, propenyl, hydroxyethyl, amidoethyl, carboxypropyl, sulfoethyl, 4-sulfonylbutyl, 2-[2-(3-sulfopropoxy)ethoxy]ethyl, propylenesulfate group or a group as described in "Zeitschrift fuer Wissenschaftliche Photographie" 63, 149 - 158, 1969, written by E. J. Poppe, X<sup>-</sup> represents an anion as is used in the synthesis of cyanine dyes, such as a bromine ion, iodide ion, p-toluenesulfonate anion, perchlorate anion, etc., p represents 1 or 2, and, when an internal salt is formed, p represents 1.

Compounds represented by general formula II are described, for example, in French Pat. No. 1,596,673. Specific examples thereof include the following compounds:

Compounds represented by General formula III can be prepared according to the procedures in U.S. Pat. Nos. 2,503,776 and 3,177,210, British Pat. No. 742,112 and German Pat. Nos. 1,072,765 and 1,163,671.

The additive amounts of the compounds of General formulae II or III are same as those for the compounds of General formula



15



5



10



15



20



25



30



35



40



45



50

Specific Examples of compounds within general formula III include the following compounds:









The silver halide emulsion used in the present invention can be silver chloride, silver bromide, silver iodide or a mixture thereof. In particular, silver chlorobromoisiodide emulsions comprising silver chlorobromide and less than 2 mole percent of iodide ions are preferred. Furthermore, silver halide emulsions comprising grains whose mode size is less than 0.8 micron and which contain at least 50 mole percent chloride ions as grain-forming ingredients are suitable. Usually the mode size is in the range 0.04-0.8 microns, preferably 0.2-0.8 microns.

Preferred emulsions for use in the present invention have a silver halide grain size of 0.1-1 micron, and contain 30-150 g per 1 mol of silver halide of a hydrophilic colloid material. The most preferred hydrophilic colloid material is gelatin. There are merely preferred embodiments, of course, and should not be construed as limiting the invention.

In the emulsion, one or more hydrophilic colloidal materials are used as a dispersing agent, and the exact material selected is not overly critical, i.e., materials such as gelatin, gelatin derivatives such as phthaloylated gelatin or malonylated gelatin, cellulose derivatives such as hydroxyethyl cellulose or carboxymethyl cellulose, soluble starches such as dextrin or alkalified starch, hydrophilic high molecular weight polymers such as polyvinyl alcohol, polyvinyl pyrrolidone, polyacrylamide or polystyrenesulfonic acid, and like materials may be used.

The emulsions can be chemically sensitized according to any process known to the art such as sulfur sensitization, reduction sensitization, sensitization with noble metal ions, e.g., a gold compound, a platinum compound, etc., or a combination of such processes. In addition, metal ions other than silver ions, such as group VIII metal ions and group II metal ions can be used to make the gradation more contrasty, to stabilize the emulsion, to control the formation of fog and to supersensitize the emulsion.

The emulsions can have added thereto a stabilizer (e.g., a 4-hydroxy-1,3,3a-7-tetrazaindene derivative), an antifogging agent, a hardener, a surfactant, a hydrophilic synthetic polymer, a latex polymer and a dye for preventing irradiation, all of which materials are commonly used in the production of light-sensitive materials.

The compounds of general formula (I) used in the invention is preferably used at a level of from about  $10^{-6}$  to about  $10^{-3}$  moles per 1 mole of silver halide. The polyalkylene oxide derivative is preferably added in an amount of from about 0.01 to 1 g per 1 mole of silver halide. Optimum results are achieved within these ranges.

In case of adding the compound to an adjacent layer

such as an overcoat layer, a backing layer, an antihalation layer, an intermediate layer or a silver halide layer, the amount of the compound is based on the silver halide contained in the silver halide emulsion layer into which the compound is diffused from the adjacent layer.

The compound of general formula (I) and the polyalkylene oxide derivatives can be added by dissolving them in water, water-miscible alcohols (e.g., methanol, ethanol, methyl cellosolve, etc.), or ketones (e.g., acetone, etc.), and then either directly added to the emulsion or added to an adjacent layer to form a multi-layer structure.

A completed emulsion in accordance with the present invention is applied to a suitable support such as a glass plate, cellulose acetate film, cellulose acetate butyrate film, polyester film or like plastic film, etc., for use. While paper can be used, it is not used in commercial practice.

An antihalation layer or a filter layer may be provided on or under the emulsion layer in accordance with the invention.

The silver halide high-sensitive material obtained by the present invention may be processed in any conventionally known manner. In development there is used, for example, an infectious developer. Such infectious developer fundamentally comprises dihydroxybenzene (developing agent), alkali, a small amount of sulfite, and sulfite ion buffer.

The developing agent, dihydroxybenzene can be selected from those known in the field of photography. Specific examples thereof include hydroquinone, chlorohydroquinone, bromohydroquinone, isopropylhydroquinone, toluhydroquinone, methylhydroquinone, 2,3-dichlorohydroquinone, 2,5-dimethylhydroquinone, etc. Hydroquinone is particularly preferred. These developing agent may be used singly or as combinations thereof.

A sulfite ion buffer is used in sufficient amount to effectively maintain the sulfite level in the developer low. Illustrative of such materials are aldehyde-alkali hydrogen sulfite adducts such as a formalin-sodium hydrogen sulfite adduct, ketone-alkali hydrogen sulfite adducts such as acetone-sodium hydrogen sulfite adducts, carbonyl bisulfite-amine condensation products such as sodium bis(2-hydroxyethyl)aminomethanesulfonate, and the like.

The developing agent, or agents, are used in amounts as are commonly used with prior art infectious developers, e.g., about 5 to about 50 g of developing agent or agents per l of developer, preferably 10-30 g per liter of developer.

The same can generally be said for the sulfite ion buffer, and such materials are generally used in an amount

of from about 13 to about 130, preferably 30-60, g per liter of developer.

An alkali material is added so as to render the developer, alkaline, preferably to a pH above 9. The type of alkali is not limited, and any of those commonly used in the photographic arts can be used for this purpose, e.g., carbonates such as potassium, sodium or calcium carbonate, etc., borax, and secondary or tertiary phosphates such as disodium phosphate, trisodium phosphate, etc.

The developer may further contain various additives known to those skilled in the art, such as an organic antifogging agent, e.g., benzotriazole, 1-phenyl-5-mercaptopurine, etc., polyalkylene oxides, amine compounds, organic solvents, e.g., triethylene glycol, dimethylformamide, methanol, ethylene glycol mono-alkyl ether, etc., and the like.

By using the light-sensitive material in accordance with the invention, there can be obtained high contrast gradation with good tone-gradation without the necessity of a comparatively long development as in the processing of conventional silver halide light-sensitive material wherein a polyalkylene oxide derivative is used. In addition, there can be obtained the effect that the quality of individual dots is uniform.

The present invention will now be described in greater detail by reference to several non-limiting Examples.

#### EXAMPLE I

A chemically ripened silver chlorobromoiodide gelatin emulsion (14 g gelatin/mole silver halide) was prepared in a conventional manner, i.e., by adding aqueous solutions of silver nitrate and potassium halide to an aqueous solution of gelatin, physically ripening it, and then adding a gold salt and sodium thiosulfate to the mixture. The bromide ion content and the iodide ion content in the emulsion were 17 mole percent and 0.2 mole percent, respectively. The amount of silver per 1 kg of the emulsion was about 1.3 moles, and the mode size of the silver halide grains was 0.6 micron. 700 g portions of the resulting emulsion were weighed out in 20 pots. Each emulsion was prepared according to the prescription given in Table 1. Preparation was as follows: first, each pot was heated to 45°C with stirring:

1. the spectral sensitizing dye was added,

2. one compound selected from the group consisting of the compounds represented by general formula (I) was added, and

3. the polyalkylene oxide derivative was added.

Table 1

| Sample No. | Sensitizing dye | Compound of general formula (I) |                                                                | Polyalkylene oxide derivative |                          |
|------------|-----------------|---------------------------------|----------------------------------------------------------------|-------------------------------|--------------------------|
|            |                 | Com-<br>ound                    | Added<br>amount<br>ml<br>(mole con-<br>centration<br>per ml.)* | Com-<br>ound                  | Added<br>amount<br>ml*** |
| 1          | —               | —                               | —                                                              | —                             | —                        |
| 2          | —               | —                               | —                                                              | (1)                           | 20                       |
| 3          | (B)             | 50<br>(5×10 <sup>-3</sup> )     | —                                                              | (1)                           | do.                      |
| 4          | (B)             | do.                             | I-2                                                            | 20                            | (1)                      |
| 5          | (B)             | do.                             | I-2                                                            | 40                            | (1)                      |
| 6          | (B)             | do.                             | I-25                                                           | 20                            | (1)                      |
| 7          | (B)             | do.                             | do.                                                            | 40                            | (1)                      |
| 8          | —               | —                               | —                                                              | (2)                           | do.                      |

Table 1-Continued

| Sample No. | Sensitizing dye | Compound of general formula (I) |                                                                | Polyalkylene oxide derivative |                          |
|------------|-----------------|---------------------------------|----------------------------------------------------------------|-------------------------------|--------------------------|
|            |                 | Com-<br>ound                    | Added<br>amount<br>ml<br>(mole con-<br>centration<br>per ml.)* | Com-<br>ound                  | Added<br>amount<br>ml*** |
| 10         | 9 (C)           | 30<br>(2×10 <sup>-3</sup> )     | —                                                              | —                             | (2) do.                  |
| 10         | 10 (C)          | do.                             | I-5                                                            | 20                            | (2) do.                  |
| 11         | 11 (C)          | do.                             | do.                                                            | 40                            | (2) do.                  |
| 12         | 12 (C)          | do.                             | I-22                                                           | 20                            | (2) do.                  |
| 13         | 13 (C)          | do.                             | do.                                                            | 40                            | (2) do.                  |
| 14         | —               | —                               | —                                                              | (3)                           | 12                       |
| 15         | 15 (A)          | 50<br>(5×10 <sup>-3</sup> )     | —                                                              | —                             | (3) do.                  |
| 16         | 16 (A)          | do.                             | I-29                                                           | 20                            | (3) do.                  |
| 17         | 17 (A)          | do.                             | do.                                                            | 40                            | (3) do.                  |
| 18         | 18 (A)          | do.                             | —                                                              | —                             | (1) 20                   |
| 19         | 19 (A)          | do.                             | I-2                                                            | 40                            | (1) do.                  |
| 20         | —               | —                               | I-2                                                            | 40                            | (1) do.                  |

In the above Table:

25 A. 1-ethyl-3-ethyl-5-(3-sulfopropyl-2-benzoxazoliniden)ethylidene-2-thiohydantoin.

B. anydro-11-ethyl-3,3'-bis(sulfopropyl)-naphtho-[1,2-d]-thiacarbocyanine hydroxide,

C. 9-methyl-3,3'-bis-(sulfobutyl)-selenacarbocyanine hydroxide,

1. polyethylene oxide derivative containing about 50 ethylene oxide chains per oleylphenoxy group, molecular weight about 2,600,

35 2. polyethylene oxide derivative containing about 30 ethylene oxide chains per oleyl alcohol group, molecular weight about 1,500,

40 3. polyalkylene oxide derivative of a block copolymer having a molecular weight of about 2,000 and comprising polypropylene oxide chains and polyethylene oxide chains, the number ratio of propylene oxide groups to ethylene oxide groups in the molecule being about 30 : 8,

45 4. ethylene oxide derivative containing about 60 ethylene oxide chains per oleylphenoxy group, molecular weight about 3,500.

\*Molar concentration and the amount of the methanol solution of the sensitizing dye added are shown.

\*\*A methanol solution of  $5 \times 10^{-3}$  molar concentration per ml was used.

\*\*\*0.5 percent by weight aqueous solution was used.

10 cc of a 1 percent aqueous solution of sodium dodecylbenzenesulfonate and 10 cc of a 2 percent aqueous solution of the sodium salt of 6-hydroxy-2,4-dichloro-S-triazine were added to each of the thus obtained emulsions as coating aids, and the emulsion obtained then applied to cellulose triacetate film in a dry thickness of about  $4\mu$  and then dried.

60 The coated film was cut into strips, and the resulting strips were wedge exposed using a 2,854°K light source by means of a sensitometer for one section (250 lux). The exposed strips were developed with the use of the following developer as is commonly employed in the development of lithographic light-sensitive materials at 20°C for 1.5 minutes, 3 minutes or 4 minutes, and then fixed.

65 Composition of the developer:

|                          |      |        |
|--------------------------|------|--------|
| Water (about 30°C)       | 500  | cc     |
| Anhydrous sodium sulfite | 30   | g      |
| Paraformaldehyde         | 7.5  | g      |
| Sodium bisulfite         | 2.2  | g      |
| Boric acid               | 7.5  | g      |
| Hydroquinone             | 22.5 | g      |
| Potassium bromide        | 1.6  | g      |
| Water to make            | 1    | liter. |

The density of the strips thus processed was measured to obtain the characteristic curves of the strips. 10 The results are shown in Table 2.

dot image having the following average density by means of a micron densitometer having an aperture  $2\mu$  width  $\times 10\mu$ , starting from the side of low density.

|                  | Average density | Dot quality |
|------------------|-----------------|-------------|
| FIG. 2, curve    | 0.40            | D           |
| FIG. 3, curve 32 | 0.38            | C           |
| FIG. 3, curve 31 | 0.40            | B           |
| FIG. 4, curve 41 | 0.37            | B           |
| FIG. 4, curve 42 | 0.37            | A           |

Table 2

| Developing time:<br>Sample | Relative sensitivity |        |        | Contrast ( $\gamma$ ) |                   |        | Dot quality |        |        | Remarks                           |
|----------------------------|----------------------|--------|--------|-----------------------|-------------------|--------|-------------|--------|--------|-----------------------------------|
|                            | 1.5 min.             | 3 min. | 4 min. | 1.5 min.              | 3 min.            | 4 min. | 1.5 min.    | 3 min. | 4 min. |                                   |
| 1                          | 5.6                  | 12.3   | 15.5   | 6                     | 5 <sup>1)</sup>   | 5      | C           | D      | D      | <sup>1)</sup> FIG. 2              |
| 2                          | —                    | 1.8    | 3.1    | —                     | 8 <sup>2)</sup>   | >13    | D           | C      | C      | <sup>2)</sup> FIG. 3              |
| 3                          | —                    | 5.2    | 6.3    | —                     | 8                 | 12     | D           | C      | C      | Curve 32                          |
| 4                          | 1.4                  | 9.1    | 15.1   | 8                     | 9                 | 13     | C           | B      | B      |                                   |
| 5                          | 2.4                  | 13.8   | 27.6   | 10                    | >13               | 8      | B           | A      | C      |                                   |
| 6                          | 2.6                  | 19.0   | 31.6   | 10                    | 10                | 10     | B           | A      | A      |                                   |
| 7                          | 6.0                  | 18.6   | 36.4   | 11                    | >13               | 6      | B           | A      | B      |                                   |
| 8                          | —                    | 1.8    | 4.0    | —                     | 10                | >13    | D           | C      | B      |                                   |
| 9                          | —                    | 1.5    | 3.1    | —                     | 4                 | >13    | D           | D      | D      |                                   |
| 10                         | 1.5                  | 10.0   | 17.4   | 7                     | >13               | >13    | D           | B      | B      |                                   |
| 11                         | 2.4                  | 14.8   | 28.1   | 12                    | 8                 | 8      | B           | B      | B      |                                   |
| 12                         | —                    | 3.8    | 10     | —                     | 7                 | >13    | D           | B      | B      |                                   |
| 13                         | 1.6                  | 12.6   | 28.2   | >13                   | 6                 | 7      | D           | B      | B      |                                   |
| 14                         | —                    | 1.3    | 2.5    | —                     | 7                 | >13    | D           | D      | B      |                                   |
| 15                         | 8.5                  | 31.6   | 56.4   | >13                   | >13 <sup>3)</sup> | 7      | D           | B      | B      | <sup>3)</sup> FIG. 1,<br>Curve 11 |
| 16                         | 21.4                 | 32.6   | 62.5   | >13                   | >13 <sup>4)</sup> | 10     | A           | A      | B      | <sup>4)</sup> FIG. 1,<br>Curve 12 |
| 17                         | 8.0                  | 30.0   | 40.0   | >13                   | >13               | >13    | A           | A      | A      | <sup>5)</sup> FIG. 5,<br>Curve 41 |
| 18                         | 7.9                  | 10.5   | 14.5   | >13                   | >13 <sup>5)</sup> | >13    | C           | B      | C      | <sup>6)</sup> FIG. 4,<br>Curve 42 |
| 19                         | 20.9                 | 48.0   | 89.0   | >13                   | >13 <sup>6)</sup> | 7      | A           | A      | B      | <sup>7)</sup> FIG. 3,<br>Curve 31 |
| 20                         | 3.5                  | 9.5    | 18.7   | >13                   | 9 <sup>7)</sup>   | 6      | A           | B      | B      |                                   |

In the Table 2, the relative sensitivity is shown in terms of the relative value of the reciprocal of the exposure amount corresponding to the point in the characteristic curve where the optical density is 0.5. Contrast is indicated in terms of average slope ( $\bar{\gamma}$ ) at the linear part of the characteristic curve. “—” means that the value was too small to measure with accuracy, while “>13” means that the value was too large to measure with accuracy, though at least higher than 13.

The rating of dot quality was determined by closely placing a contact screen (133 line/1 inch) on a sample and exposing and developing the sample in the same manner as above, and observing the thus obtained dot image with an optical microscope. The samples were classified into four equally spaced grades, A (best), B, C and D, (worst-impractical for use) in the order of the sharpness of their dot edges.

The results of this rating method approximately coincided with the order of height of the edge gradient obtained by measuring the micron density of the dot image by means of a micron densitometer.

In FIGS. 2 – 4 curves showing the relationship between distance and optical density with respect to the edge portions are given, the relationship being based on 65 the average of six dots.

These were obtained by measuring the density of a

Curve 51 in FIG. 5 shows the range of individual curves used to obtain curve 41 in FIG. 4, and curve 52 in FIG. 5 shows the range with the curve in FIG. 4. It can be understood that the quality of the individual dots was made uniform by the presence of the compound of the general formula (I) in accordance with the invention.

Studying the results given in Table 2 in detail, it can be seen that with the silver halide light sensitive material containing neither the compound represented by general formula (I) nor the sensitizing dyes represented by the general formula II or III, i.e., containing only a polyalkylene oxide derivative, there is the tendency that the longer the developing time the higher both the relative sensitivity and contrast become, and the more improved the dot quality becomes (see Samples 2, 8 and 14).

Further in the case of adding the sensitizing dye represented by general formula II or III and not adding the compound represented by general formula I, as the developing time increased the sensitivity increased. However, in this case there was not great change in the contrast (see Sample 3) and, in some cases, a detrimental effect was encountered (see Sample 9). Although there were the cases wherein both sensitivity and contrast were good as in Samples 15 and 18, the dot quality can-

not be said to be improved in proportion to sensitivity and contrast.

However, it can be seen that by utilizing a system within the present invention there was obtained an excellent, high contrast light-sensitive material having higher sensitivity than that of any of the conventional materials which provided good dot quality. (For example, compare Sample 19 or 20 in accordance with the present invention with Sample 18, a comparison sample).

### EXAMPLE 2

A chemically ripened silver chlorobromide gelatin emulsion (74 g gelatin/mole silver halide) was prepared in a conventional manner as in Example 1. The bromide ion content in the emulsion was 30 mole percent, and the amount of silver per 1 kg of the emulsion was about 1.1 moles.

Samples of the light-sensitive material was prepared according to Example 1 under the conditions given in Table 3, and subjected to sensitometry as in Example 1. The results shown in Table 3 were obtained.

The terms in Table 3 have the same meaning as in Tables 1 and 2.

10

5

15

20

25

Table 3

| No. | Compound of general formula (I) | Amount (cc) (Molar conc.)     | Poly-alkylene oxide derivative | Amount (cc) (% by wt.) | Relative sensitivity | Contrast ( $\gamma$ ) |             |        |         |         |        | Dot quality |
|-----|---------------------------------|-------------------------------|--------------------------------|------------------------|----------------------|-----------------------|-------------|--------|---------|---------|--------|-------------|
|     |                                 |                               |                                |                        |                      | 1'30"                 | 3'          | 4'     | 1'30    | 3'      | 4'     | 1'30"       |
| 21  | —                               | —                             | —                              | —                      | 6.0<br>1.4           | 12.5<br>2.0           | 16.2<br>3.1 | 6<br>6 | 5<br>11 | 4<br>11 | D<br>D | B<br>B      |
| 22  | —                               | 4                             | —                              | 20<br>(0.5%)           | —                    | —                     | —           | —      | —       | —       | —      | —           |
| 23  | I-19                            | 100<br>( $2 \times 10^{-3}$ ) | 4                              | do.                    | 2.4                  | 12.6                  | 24.0        | >13    | >13     | 7       | B      | A           |
| 24  | I-2                             | 50<br>( $2 \times 10^{-3}$ )  | 4                              | do.                    | 1.9                  | 8.0                   | 15.9        | 10     | >13     | 8       | B      | A           |
| 25  | do.                             | 100<br>( $2 \times 10^{-3}$ ) | 4                              | do.                    | 2.3                  | 9.5                   | 16.0        | 10     | >13     | 8       | B      | A           |
| 26  | do.                             | 150<br>( $2 \times 10^{-3}$ ) | 4                              | do.                    | 2.8                  | 9.3                   | 17.8        | >13    | >13     | 7       | A      | A           |
| 27  | I-39                            | 50<br>( $2 \times 10^{-3}$ )  | 4                              | do.                    | 3.6                  | 14.0                  | 1.58        | >13    | 11      | 6       | A      | B           |
| 28  | do.                             | 100<br>( $2 \times 10^{-3}$ ) | 4                              | do.                    | 2.7                  | 12.1                  | 18.8        | >13    | 8       | 6       | A      | B           |
| 29  | do.                             | 150<br>( $2 \times 10^{-3}$ ) | 4                              | do.                    | 3.0                  | 11.2                  | 16.0        | >13    | 7       | 6       | A      | B           |
| 30  | I-18                            | 100<br>( $2 \times 10^{-3}$ ) | 4                              | do.                    | 1.1                  | 2.0                   | 6.8         | 6      | >13     | >13     | B      | B           |
| 31  | do.                             | 150<br>( $2 \times 10^{-3}$ ) | 4                              | do.                    | 1.6                  | 2.4                   | 7.1         | 7.1    | >13     | >13     | B      | A           |

From the results shown in Table 3 it can be seen that according to the present invention dots having good quality and high sensitivity can be obtained with a short development.

Preferred embodiments of the present invention are as follows.

1. In the invention, a silver halide emulsion spectrally sensitized with a sensitizing dye represented by the general formula (II) or (III) is used.

2. In the invention, an emulsion containing silver halide grains of less than 0.8 micron in grain mode size and comprising at least 50 mole percent silver chloride are used.

While the invention has been described in detail and with reference to specific embodiments thereof, it will be apparent to one skilled in the art that various changes and modifications can be made therein without departing from the spirit and scope thereof.

What is claimed is:

1. A silver halide light-sensitive material which comprises in a silver halide emulsion layer or a layer adjacent thereto at least one heterocyclic thioketone compound which does not form a mercapto group through tautomerism, said compound being represented by the following general formula (I):



wherein Q represents the group of atoms necessary to form a heterocyclic ring selected from the group consisting of benzothiazoline-2-thione ring, benzoselenazolin-2-thione ring, benzoxazolin-2-thione ring, imidazolin-2-thione ring, benzimidazolin-2-thione ring, selenazolidin-2-thione ring, 4-selenazolin-2-thione ring, 1,3,4-thiodiazolin-2-thione ring, 1,3,4-

50 selenadiazoline-2-thione ring, 1,2-dihydropyridin-2-thione ring, 1,2-dihydroquinolin-2-thione ring, 4,5-tetramethylenethiazolin-2-thione ring, 4,5-trimethylenethiazoline-2-thione ring, naphthothiazolin-2-thione ring, and thiazolidin-2-thione ring, and R represents an unsubstituted alkyl group, an aralkyl group 55 an aryl group, a 2-pyridyl group or a dipyrindyl group and at least 1 polyalkylene oxide derivative having a molecular weight ranging from 500 to 12,000 selected from the group consisting of

- block copolymers of alkylene oxide,
- polyalkyleneglycols,
- addition polymerization products between alkylene oxides and a compound selected from the group consisting of an aliphatic alcohol, an aromatic alcohol, glycols, fatty acids, organic amines, and a dehydrated compound of hexitol derivatives, and

60

65

d. condensates of a polyalkylene oxide with said compound, the combination of said thioketone compound and said polyalkylene oxide derivative being incorporated in said layer in concentrations which provide a high edge gradient with comparatively short development time and/or dots having good toe-gradation when said material is developed.

2. The silver halide light-sensitive material of claim 1 wherein the silver halide has a mode grain size of 0.2 to 0.8 microns.

3. The silver halide light-sensitive material of claim 1 wherein the silver halide emulsion layer comprises a hydrophilic colloid.

4. The silver halide light-sensitive material of claim 1 wherein the compound of general formula (I) is present in an amount of from about  $10^{-6}$  to about  $10^{-3}$  moles and the polyalkylene oxide derivative is present in an amount of from about 0.01 to about 1 g per mole of silver halide in the silver halide emulsion layer.

5. The silver halide light-sensitive material of claim 1 wherein R is an unsubstituted alkyl group of 1-13 carbon atoms.

6. The silver halide light-sensitive material of claim 1 wherein R is an aryl group.

7. The silver halide light-sensitive material of claim 1 wherein R is a 2-pyridyl group or a dipyridyl group.

8. The silver halide light-sensitive material of claim 1 wherein R is selected from group consisting of a methyl group, ethyl group, propyl group, hexyl group, decyl group, and a benzyl group.

9. The silver halide light-sensitive material of claim 6 wherein R is selected from the group consisting of a phenyl group, 2-methylphenyl group, 4-methoxyphenyl group and a 4-chlorophenyl group.

10. The silver halide light-sensitive material of claim 1 wherein the polyalkylene oxide derivative is selected

from the group consisting of

a.



b.



c.



wherein b represents an integer of 14-55 and a+c is an integer of 4-210.



e.



30 wherein  $l+m+n =$  about 20, and

f.



\* \* \* \* \*